

March 7, 1950

J. A. M. SMELT

2,499,789

METHOD OF MANUFACTURING MAGNETIC MASS CORES

Filed Sept. 19, 1945



JOSEPHUS ANTONIUS MARIA SMELT  
INVENTOR.

BY

ATTORNEY.

## UNITED STATES PATENT OFFICE

2,499,789

METHOD OF MANUFACTURING MAGNETIC  
MASS CORESJosephus Antonius Maria Smelt, Eindhoven,  
Netherlands, assignor to Hartford National  
Bank & Trust Co., Hartford, Conn., as trusteeApplication September 19, 1945, Serial No. 617,453  
In the Netherlands June 16, 1942Section 1, Public Law 690, August 8, 1946  
Patent expires June 16, 1962

7 Claims. (Cl. 25—156)

1

It is known to manufacture magnetic mass cores, for example for radio and telephony purposes, by moulding, if necessary with the aid of a binding agent, a finely divided magnetic metal powder in a matrix at high pressure and, if desired, at increased temperature to form the shape of core desired.

It is further known to form a core by moulding powdery magnetic insulating materials, as magnetite or other ferrites, for example copper ferrite, with the aid of a binding agent in a matrix. For the chemical preparation of these ferrites a mixture of the oxides constituting the ferrite is usually compressed to form a block or a rod, the compressed mixture of oxides being sintered until it has changed to ferrite, whereafter pulverisation takes place.

Another method of manufacturing magnetic cores consists in extrusion moulding in a matrix a mixture of a powder of magnetic material with a binding agent which is fluid under the influence of heat and solidifies during cooling down in the matrix.

The present invention relates to a method of manufacturing magnetic mass cores, which is superior to all previous methods as regards simplicity and quickness of manufacture. It relates more particularly to a method of manufacturing mass cores which comprise ferrite as a magnetisable material.

According to the invention, the shaping of such cores is effected with the aid of an extrusion press and for the purpose of obtaining sufficient coherence of the extruded material, the material to be pressed is additioned by an organic binding agent or an adhesive, as potato flour, wheat flour, tragacanth, nitrocellulose.

It is thus possible, for example, for a powdery ferrite additioned by an organic binder to be moulded by means of an extrusion press to form a string of the desired section of core and for the string to be cut into pieces and subsequently heated until the ferrite particles sinter together. Since during this heating the organic binding agent is expelled, the material after the heating contains no foreign non-magnetic substances which might impair the permeability of the core.

Cores thus manufactured, which may be either hollow or solid and may exhibit a circular, rectangular or any other section, are of a uniform structure. If desired, they may be subsequently ground to the correct size.

The present invention is particularly advantageous in the manufacture of elongated magnetic cores for which it was hitherto difficult to ob-

2

tain a uniformly magnetic structure throughout their length.

According to the invention, it has further been found that a mixture of oxides of the kind as is ordinarily used for the chemical preparation of a magnetic ferrite is very suitable to be moulded by means of an extrusion press. This fact is taken into account in one embodiment of the invention in which a powdery mixture of oxides additioned by an organic binding agent is moulded with the aid of an extrusion press to form a string of the desired section of core, after which a heating takes place, during which the mixture of oxides changes into the corresponding magnetic product.

Relatively to the method of manufacture in which the completed magnetic product previously sintered is moulded, the above-mentioned special method offers the advantage that a mixture of oxides is softer than the sintered product, which is of importance for moulding. Another advantage consists in that the shaping of the core and the chemical preparation of the magnetisable product are in this case combined in one operation in contradistinction to the first-mentioned method of manufacture in which a magnetic product prepared in a special chemical process is moulded to form a core and sintered. This means a considerable simplification, since now only one heating takes place and only the soft mixture of oxides has to be ground, the grinding of the harder product specially manufactured, which grinding takes much time, being suppressed.

For completeness' sake it is mentioned that the mixture of oxides, which may also contain hydroxides, which is used as a primary material in the chemical preparation of a magnetic ferrite, may be either of a stoichiometrical composition or of a composition different therefrom; the ferrioxide or hydroxide may in this case be mixed either with a simple metallic oxide or with a mixture of several metallic oxides. It is also possible to substitute aluminium oxide or chromium oxide for part of the ferrioxide whilst retaining the ferrite crystal structure of the sintered magnetic product.

The following example describes the manufacture of a magnetic core constituted by a mixed copper-zinc ferrite. As a rule, mixtures of oxides which are constituted by ferrioxide, zinc oxide and one or a plurality of other oxides and which change into a mixed zinc ferrite during sintering may be excellently moulded by means of an extrusion press.

**3**  
*Example*

250 g. of a mixture composed of 20 mol. per cent of copper oxide, 30 mol. per cent of zinc oxide and 50 mol. per cent of ferrioxide are mixed with 45 g. of a solution of 18% by weight of nitrocellulose in a solvent composed of 50 parts of butyl acetate, 25 parts of butanol and 15 parts of ethyl glycol. With the aid of an extrusion press the mixture is moulded to form a tube having an external diameter of 4.8 mms. and an internal diameter of 2.5 mms. After sintering during 2 hours at 1150° C., a magnetic tubular core of copper-zinc ferrite is obtained having an external and an internal diameter of 4 mms. and 2 mms. respectively.

In order that the invention can be more readily understood and carried into effect it will now be described with reference to the accompanying drawing in which an extrusion mold for extruding a core according to the invention is illustrated.

Referring more particularly to the figure, an extrusion mold 1 is adapted to hold a mixture of ferrite material and an organic binding agent 2 extrudes a compact core 3 through a reduced portion of the mold 4 when plunger 5 compresses the mixture 2.

What I claim is:

1. The method of manufacturing a ferromagnetic core comprising the steps of adding an organic binder to powdered ferrite-forming constituents, extruding the ferrite-forming constituents containing the organic binder to form a core, and sintering said core at a temperature of about 1150° C. to form a mixed ferrite and to expel said binder and form a compact core of ferrite material.

2. The method of manufacturing a ferromagnetic core comprising the steps of, mixing a powdered metallic oxide, powdered zinc oxide, and powdered iron oxide, adding an organic binder to said powdered oxide, extruding the oxide mixture containing the organic binder to form a core, and sintering said core at a temperature of about 1150° C. to form a mixed ferrite and to expel said binder.

3. The method of manufacturing a ferromagnetic core comprising the steps of, adding potato flour to powdered metal oxide ferrite-forming constituents, extruding the oxide constituents containing potato flour to form a core, and sintering said core at a temperature of about 1150° C. to form a mixed ferrite and to expel the potato flour.

4. The method of manufacturing a ferromag-

**4**

netic core comprising the steps of, adding wheat flour to powdered metal oxide ferrite-forming constituents, extruding the oxide constituents containing wheat flour to form a core, and sintering said core at a temperature of about 1150° C. to form a mixed ferrite and to expel the wheat flour.

5. The method of manufacturing a ferromagnetic core comprising the steps of, adding tragacanth to powdered metal oxide ferrite-forming constituents, extruding the oxide constituents containing tragacanth to form a core, and sintering said core at a temperature of about 1150° C. to form a mixed ferrite and to expel the tragacanth.

6. The method of manufacturing a ferromagnetic core comprising the steps of, adding nitrocellulose to powdered metal oxide ferrite-forming constituents, extruding the oxide constituents containing nitrocellulose to form a core, and sintering said core at a temperature of about 1150° C. to form a mixed ferrite and to expel the nitrocellulose.

7. The method of manufacturing a ferromagnetic core comprising the steps of, mixing powdered copper oxide, powdered zinc oxide, and powdered iron oxide, in approximate molecular percentages of 20:30:50 respectively, adding a solution of 18% of weight of nitrocellulose in a solvent of butyl acetate, butanol, and ethyl glycol in the approximate ratio of 50:25:15 to said powdery mixture, extruding said powdery mixture containing nitrocellulose in said solvent to form a core, and heating said core at a temperature of approximately 1150° for approximately 2 hours to form a mixed copper-zinc ferrite and to expel said nitrocellulose and said solvent.

JOSEPHUS ANTONIUS MARIA SMELT.

**REFERENCES CITED**

The following references are of record in the file of this patent:

**UNITED STATES PATENTS**

|    | Number    | Name      | Date          |
|----|-----------|-----------|---------------|
| 45 | 1,292,206 | Woodruff  | Jan. 21, 1919 |
|    | 1,669,548 | Elmen     | May 15, 1928  |
|    | 1,669,646 | Bandur    | May 15, 1928  |
|    | 1,807,915 | Iredell   | June 2, 1931  |
| 50 | 1,899,584 | Novias    | Feb. 28, 1933 |
|    | 1,904,273 | Crowley   | Apr. 18, 1933 |
|    | 1,946,964 | Cobb      | Feb. 13, 1934 |
|    | 2,031,129 | Reichmann | Feb. 18, 1936 |
|    | 2,134,752 | Ehlers    | Nov. 1, 1938  |